

106-18,27

C222A

XR

SR

2,305,325

27

Filed in 106-18,26

3/21/86

45

Dec. 15, 1942.

P. M. SNYDER

2,305,325

INSULATED WIRE

Filed Aug. 23, 1941

Fig. 1

Fig. 2



BY

INVENTOR

Peter M. Snyder  
J. Stanley Sherschell  
Atty.

3-15% 2,305,325

by way of the

see claim 1 A.C.  
14

## UNITED STATES PATENT OFFICE

2,305,325

## INSULATED WIRE

Purdum M. Snyder, Ben Avon, Pa., assignor to  
H. H. Robertson Company, Pittsburgh, Pa., a  
corporation of Pennsylvania

Application August 23, 1941, Serial No. 408,134

12 Claims. (CL. 174—120)

This invention relates to rubber covered insulated wire.

In general, the object of the invention is to produce a novel and improved rubber coated insulated wire which may be economically manufactured, possesses the general physical characteristics as to flexibility, maintenance of its insulating characteristics over long periods of time, and other general characteristics comparable to the rubber covered insulated wire now upon the market, and which in addition possesses the ability to retard propagation of flame when the wire is subjected to the direct action of a fire.

With this general object in view, and such others as may hereinafter appear, the invention consists in the flame retarding rubber covered insulated wire hereinafter described and particularly defined in the claims at the end of this specification.

In the drawing, Fig. 1 illustrates a length of a rubber covered insulated wire embodying the invention, and Fig. 2 is a cross-section on the line 2—2 of Fig. 1. In accordance with the usual process which has heretofore been employed in the production of rubber covered insulated wire, the copper wire 10 is preferably provided with a coating of tin 12, and the rubber insulation 14 may be applied directly over the tin coating by an extrusion process, by being wrapped about the wire, or in any other suitable manner. Thereafter a cotton braid or similar textile covering is wrapped or served over the rubber insulation and the partially completed wire is then passed through an impregnating bath of a bituminous material to weatherproof and saturate the textile covering 18. After the wire has been thus saturated with the bituminous impregnant, it may be immediately finished, or in accordance with the usual practice, such wire is permitted to cool, and in either instance is wiped to remove the surplus impregnant from the surface thereof and then passed through a bath of a bituminous finishing composition to apply a finishing coating 20 thereto. In some instances it may be desirable to color the finishing coating as indicated by a coloring layer 22 and also to provide a lubricant in the nature of a paraffin, wax, or similar surface coating 24.

In accordance with the usual commercial practice the speed at which the insulated wire is passed through the saturating bath varies from 100 to 400 feet per minute so that the saturant or impregnant is required to be a relatively low melting point bituminous material, varying in melting point from 100 to 200° F. The usual

temperature at which saturation is conducted approximates 350° F. in order to render the bituminous impregnant or saturant sufficiently fluid to thoroughly effect the desired saturation of the braid or similar textile layer during the passage of the wire through the bath at the relatively high speed of from 100 to 400 feet per minute. In practice, it has been found that bituminous materials are satisfactory having a hardness or penetration of from 15 to 30 when tested at 77° F. using 100 grams for 5 seconds, in accordance with the standard methods of testing bituminous materials for penetration and hardness.

After the partially completed wire has been saturated and as it comes from the saturating bath, it is usually reeled up and stored to be subsequently finished, and in order to apply the finishing coat the wire is passed through a bath of the finishing composition which preferably comprises a bituminous composition having a melting point of from 170° F. to 300° F. and having a penetration or hardness within the range of from 3 to 18, and preferably within the limits of from 6 to 10 when measured using 100 grams for 5 seconds, as above described. It is preferred that the finishing composition not be too hard as otherwise a tendency to flake from the surface of the wire is experienced, and if too soft, then the wire soon gets out of shape when reeled in a coil, and further will not satisfactorily pull through the usual wiring conduits during the use of the wire in wiring buildings and the like. In order to assist the pulling of the wire through the conduits an additional lubricating coat in the nature of a wax or paraffin coat, and also if desired, an underlying color coat, may be applied to the finishing coat of the rubber covered insulated wire.

In producing the present bituminous composition possessing the desired flame retarding properties, a bituminous base is utilized and a definite proportion of a metallic soap is incorporated therein. The bituminous base may comprise any of the natural asphalts, gilsonite, steam reduced and air blown asphalts from petroleum residua, coal tar pitches and stearine pitches, and mixtures thereof. The metallic soap may comprise a soap selected from the soaps from the group of metals consisting of manganese, iron, zinc, chromium, cobalt, aluminum, magnesium, lead and barium, but best results have been secured utilizing a soap selected from the soaps from the group of metals consisting of iron, zinc, aluminum and barium. One or more soaps may be utilized in an amount within the range of from

3 to 15% by weight of the bituminous composition and preferably from 6 to 15% of such soaps.

The incorporation of these metallic soaps is preferably accomplished by mixing the previously prepared soaps, substantially free from moisture, with the bituminous composition at an elevated temperature, preferably above 150° F. or at such a temperature at which the bituminous base becomes sufficiently fluid to render the dispersion of the soap therein a simple mixing procedure. In some instances, incorporation of the soap may be caused to take place directly in the bituminous composition, such for example as by incorporating zinc oxide in a bituminous composition having blended in it a fatty acid and heating the mixture until saponification has been completed and the moisture resulting from the reaction has been dissipated. The quantity of zinc oxide added should be the amount required to satisfy the acid content and in such quantity that the total soap formed is within the prescribed limits of from 3 to 15%.

While manganese soaps impart more effective flame retardance to the bituminous compositions, nevertheless, because of the fact that manganese appears to be such an active catalyst, it is preferred for many purposes to utilize a soap or mixtures of soaps selected from the group comprising the soaps of iron, zinc, aluminum and barium, as such soaps appear to produce compounds efficient in flame retardance and at the same time of relatively permanent physical characteristics.

The present bituminous compositions possess effective flame retardance particularly useful in the production of rubber insulated cotton covered wire commonly known as code wire. Rubber insulated cotton covered wire having fire resistance and moisture proof properties is so made by first saturating the cotton braid with a stearine pitch-bearing composition, and then coating this saturated wire with a stearine pitch-bearing compound. In addition to making such wire fire resisting and moisture resisting, these stearine pitch-bearing compounds must have such physical properties so as to impart to the finished wire the ability to comply with other performance requirements such as flexibility, temperature stability and a low coefficient of friction. Typical examples of these performance requirements follow in a description of a flame test and a moisture absorption test.

#### Flame test

Support an 18" sample vertically and rigidly in a room from which all drafts are excluded. A flame indicator of gummed Kraft paper,  $\frac{1}{2}$ " wide and 5 mils thick, shall be wrapped once around the sample with its lower edge 10" above the point at which the flame is applied. The ends of the indicator shall be pasted evenly together and shall project  $\frac{3}{4}$ " on the side of the wire opposite to that on which the flame is applied.

Apply the  $\frac{1}{2}$ " blue cone of a 5" flame (from a  $\frac{1}{4}$ " Bunsen burner having  $\frac{1}{4}$ " inlet and  $\frac{3}{8}$ " to  $\frac{1}{2}$ " mouth) at an angle of 20°, approximately 3" from the bottom of the sample, for 15 seconds, then remove for 15 seconds. This process is repeated four times, after which the sample shall not continue to burn for more than one minute and the paper indicator shall not be burned more than 25% of its area.

#### Moisture absorption test

A sample shall be bent around a mandrel, the 75

diameter of which shall be determined from the overall diameter of the wire as follows:

|    | Size of conductor         | Diameter of mandrel                  | De-grees bend |
|----|---------------------------|--------------------------------------|---------------|
| 5  | 14 to 12 A. W. G.         | 1 times diameter of wire             | 360+          |
| 10 | 10 to 8 A. W. G.          | $\frac{1}{2}$ times diameter of wire | 360+          |
|    | 6 to 2 A. W. G.           | 2 times diameter of wire             | 300+          |
|    | 1 to 4/0 A. W. G.         | 3 times diameter of wire             | 180           |
|    | 250,000 to 500,000 CM     | 4 times diameter of wire             | 180           |
|    | 550,000 to 1,000,000 CM   | 6 times diameter of wire             | 180           |
|    | 1,100,000 to 2,000,000 CM | 7 times diameter of wire             | 180           |

The sample shall be immersed in distilled water at room temperature for 72 hours after which the braids shall not have absorbed more than 15% of their weight.

Stearine pitch is a by-product of the fatty acid industry and is accordingly limited in supply. In addition, because of the varying materials and conditions under which commercial forms of stearine pitches are produced, it has been increasingly difficult to obtain such pitches possessing uniform performance from a flame-retarding standpoint. It has also been found exceedingly difficult to manufacture uniform stearine pitch-bearing compounds from a physical characteristic standpoint, such as softening point, viscosity and hardness, which have a direct effect on the performance properties of such articles as rubber insulated wire, tubular woven conduits and other articles of commercial significance.

The barium soaps have been found to be particularly effective from a flame retarding standpoint. However, the barium soaps are not readily dispersed in asphalts by simple mixing and fluxing together. In an effort to find a method whereby this could be accomplished, it was found that the barium soaps could first be mixed with other soaps which were readily dispersed by simple mixing and fluxing, and then in such combination could readily be dispersed in asphalts.

It was found that 50 parts of a barium soap and 50 parts of a zinc soap when mixed together, and then added to an asphalt or a bituminous combination, that fire retarding properties approximating the effectiveness of a manganese soap could be obtained, when added in approximately the same proportions. Percentages required to produce materials of commercial value fall within the range of 4 to 12%. In practice we have found that 6 to 12% is adequate.

Rubber insulated cotton covered wire treated with bituminous materials containing this combination after 6 months exposure have not exhibited the tendency to deteriorate. The degree of deterioration appears to be of about the same magnitude as would be obtained with straight asphaltic materials.

For example, I have found that when 6% of a mixture of 50% barium laurate and 50% zinc laurate is added to an asphalt having a melting point of 140° F. ball and ring, and a penetration of 21 at 77° F. 100 grams for 5 seconds, that the resulting composition has a melting point of 140° F., and a penetration of 20 at 77° F. Viscosity at 300° F. remains the same after the soap addition. These same physical properties can be readily reproduced from batch to batch. Further the flame retarding properties of such a combination are consistent from batch to batch. For example, I have found that when rubber insulated cotton covered wire is impregnated with this material and an excess is allowed to remain on the wire, and subjected

to a 5 inch Bunsen burner flame while suspended in a vertical position, that sufficient encrusting occurs to thwart the propagation of a flame upward. A material having a melting point of 140° F., and a penetration of 20 at 77° F., is however, in itself unsuitable for the production of commercial wire, because of its tackiness and low flow point. In other words, wire finished with such a material would stick together in coils. Therefore, in practice, a material of this nature would be used solely as a saturant for the cotton braid, wiped reasonably dry, and subsequently finished with a harder, higher melting point material to render the wire suitable for handling.

I have found that when a bituminous composition composed of asphalt alone or complex bituminous mixtures such as a blend of asphalts, gilsonite, and wax, having melting points varying in range from 200 to 250° F. and penetration values varying from 3 to 15 at 77° F., has a barium and zinc soap combination incorporated therein, is suitable as a finisher for such work, and that the physical properties such as melting point and hardness is not substantially changed. Such materials fall well within the range required of coating materials used in the production of fire retarding, rubber insulated cotton covered code wire and in addition, such compounds have fire retarding properties equal to commercial forms of stearine pitch compounds used in the production of flame retarding, moisture resisting code wire.

For example, I have found that when eight per cent of a combination of 50 parts barium laurate and 50 parts zinc laurate are incorporated in an asphalt having a melting point of 238° F., and a penetration of 8 at 77° F., that the resulting melting point is 231° F., and the penetration at 77° F., is 9.

I have further found that when rubber insulated cotton wire is saturated with a 140° F. melting point bituminous composition such as described above, and subsequently finished with a finisher as cited in the above example, that this wire equals in fire resistance performance, and in some instances is superior to wire impregnated with commercial forms of stearine pitch saturants and finishers.

There are many types and sizes of rubber insulated cotton covered wire, and experience has shown that application technique with respect to saturation and finishing must be varied to make all of these various wires behave in a similar manner with respect to fire resistance.

This is true both for the stearine pitch type saturants and finishers as well as the soap types. In brief the proper technique required for each type of wire is one whereby the necessary amount of saturant and finisher can be retained in the cotton covering, so that the ash structure formed on burning is adequate to thwart the propagation of a flame. Controlling factors are the temperature of the saturating and finishing bath, the speed of the wire through these baths, and the size of the finishing dies. In certain instances it may even be necessary to double coat the wire, either by having a finishing tank in tandem with the saturating bath which puts on a light smear coat of finisher, or by running the wire through the finishing bath two times.

For some purposes I have found that combinations of several soaps may be used with advantage, particularly to obtain maximum effectiveness with respect to flame retardance. For example, it has been found that the addition of

3% iron stearate to an asphalt saturant or finisher for the production of code wire and embodying 8% of a barium zinc soap combination produces a bituminous composition which possesses very efficient flame retarding characteristics. Other soaps may be included as above described, such for example, as minor proportions of aluminum soaps, with barium and zinc soap combinations.

10 This application is a continuation in part of my application, Serial No. 183,160, filed January 3, 1938.

Having thus described the invention, what is claimed is:

15 1. As a new article of manufacture, a rubber covered insulated wire comprising a wire having a coating of rubber insulating the same, and a textile covering member applied to and covering the rubber coating, said textile covering member being impregnated with a bituminous impregnant, and having a bituminous finishing coating applied over and covering the textile covering, said bituminous finishing coating being characterized by the ability when exposed to direct 20 flame of forming a carbonaceous ash film on the surface thereof in sufficient amount to form an effective air seal to thereby prevent rapid propagation of flame, said finishing coating comprising a bituminous material selected from the 25 group consisting of those natural asphalts, gilsonite, steam reduced and air blown asphalts, from petroleum residua, coal tar pitches, stearine pitches, and mixtures thereof which are characterized by their non-greasy and non-oily appearance and feel, and having incorporated therein at least one metallic soap insoluble in water and comprising a soap selected from the soaps of the 30 group of metals consisting of iron, zinc, aluminum, and barium, in an amount not exceeding fifteen per cent by weight of the bituminous composition, said flame retarding bituminous composition being further characterized by its ability to maintain substantially predetermined 35 physical characteristics upon cooling after having been subjected to heating to elevated temperatures.

2. As a new article of manufacture, a rubber covered insulated wire comprising a wire having a coating of rubber insulating the same, and a textile covering member applied to and covering the rubber coating, said textile covering member being impregnated with a bituminous impregnant, and having a bituminous finishing coating applied over and covering the textile covering, 40 said bituminous finishing coating being characterized by the ability when exposed to direct flame of forming a carbonaceous ash film on the surface thereof in sufficient amount to form an effective air seal to thereby prevent rapid propagation of flame, said finishing coating comprising a bituminous material selected from the group consisting of those natural asphalts, gilsonite, steam reduced, and air blown asphalts from petroleum residua, coal tar pitches, stearine pitches, and mixtures thereof which are characterized by their non-greasy and non-oily appearance and feel, and having incorporated therein at least one metallic soap insoluble in water and 45 comprising a soap selected from the soaps of the group of metals consisting of iron, zinc, aluminum, and barium, in an amount not exceeding fifteen per cent by weight of the bituminous composition, said bituminous material having incorporated therein waxes, resins or mixtures thereof.

in proportions not to exceed 35% of the weight of the bituminous composition, said flame retarding bituminous composition being further characterized by its ability to maintain substantially predetermined physical characteristics upon cooling after having been subjected to heating to elevated temperatures, said bituminous material constituting at least 65% of the bituminous base.

3. As a new article of manufacture, a rubber covered insulated wire comprising a wire having a coating of rubber insulating the same, and a textile covering member applied to and covering the rubber coating, said textile covering member being impregnated with a bituminous impregnant, and having a bituminous finishing coating applied over and covering the textile covering, said bituminous finishing coating being characterized by the ability when exposed to direct flame of forming a carbonaceous ash film on the surface thereof in sufficient amount to form an effective air seal to thereby prevent rapid propagation of flame, said finishing coating comprising a bituminous material selected from the group consisting of those natural asphalts, gilsonite, steam reduced and air blown asphalts from petroleum residua, coal tar pitches, stearine pitches and mixtures thereof which are characterized by their non-greasy and non-oily appearance and feel, and having incorporated therein at least one metallic soap insoluble in water and comprising a soap selected from the soaps of the group of metals consisting of iron, zinc, aluminum and barium, in an amount from six to fifteen per cent by weight of the bituminous composition, said flame retarding bituminous composition being further characterized by its ability to maintain substantially predetermined physical characteristics upon cooling after having been subjected to heating to elevated temperatures.

4. As a new article of manufacture, a rubber covered insulated wire comprising a wire having a coating of rubber insulating the same, and a textile covering member applied to and covering the rubber coating, said textile covering member being impregnated with a bituminous impregnant, and having a bituminous finishing coating applied over and covering the textile covering, said bituminous finishing coating being characterized by the ability when exposed to direct flame of forming a carbonaceous ash film on the surface thereof in sufficient amount to form an effective air seal to thereby prevent rapid propagation of flame, said finishing coating comprising a bituminous material selected from the group consisting of those natural asphalts, gilsonite, steam reduced and air blown asphalts from petroleum residua, coal tar pitches, stearine pitches, and mixtures thereof which are characterized by their non-greasy and non-oily appearance and feel, and having incorporated therein at least one metallic soap insoluble in water and comprising a soap selected from the soaps of the group of metals consisting of manganese, iron, zinc, chromium, cobalt, magnesium, lead and barium, in an amount not exceeding fifteen per cent by weight of the bituminous composition, said flame retarding bituminous composition being further characterized by its ability to maintain substantially predetermined physical characteristics upon cooling after having been subjected to heating to elevated temperatures.

5. As a new article of manufacture, a rubber covered insulated wire comprising a wire having a coating of rubber insulating the same, and a textile covering member applied to and covering

the rubber coating, said textile covering member being impregnated with a bituminous impregnant, and having a bituminous finishing coating applied over and covering the textile covering, 5 said bituminous finishing coating being characterized by the ability when exposed to direct flame of forming a carbonaceous ash film on the surface thereof in sufficient amount to form an effective air seal to thereby prevent rapid propagation of flame, said finishing coating comprising a bituminous material selected from the group consisting of those natural asphalts, gilsonite, steam reduced and air blown asphalts from petroleum residua, coal tar pitches, stearine pitches, and mixtures thereof which are characterized by their non-greasy and non-oily appearance and feel, and having incorporated therein a mixture of barium and zinc soaps in an amount not exceeding fifteen per cent by weight of the bituminous composition, said flame retarding bituminous composition being further characterized by its ability to maintain substantially predetermined physical characteristics upon cooling after having been subjected to heating to elevated temperatures.

6. As a new article of manufacture, a rubber covered insulated wire comprising a wire having a coating of rubber insulating the same, and a textile covering member applied to and covering the rubber coating, said textile covering member being impregnated with a bituminous impregnant, and having a bituminous finishing coating applied over and covering the textile covering, 10 said bituminous finishing coating being characterized by the ability when exposed to direct flame of forming a carbonaceous ash film on the surface thereof in sufficient amount to form an effective air seal to thereby prevent rapid propagation of flame, said finishing coating comprising a bituminous material selected from the group consisting of those natural asphalts, gilsonite, steam reduced and air blown asphalts from petroleum residua, coal tar pitches, stearine pitches, and mixtures thereof which are characterized by their non-greasy and non-oily appearance and feel, and having incorporated therein a mixture of fifty per cent barium soap and fifty per cent zinc soap in an amount not exceeding fifteen per cent by weight of the bituminous composition, said flame retarding bituminous composition being further characterized by its ability to maintain substantially predetermined physical characteristics upon cooling after having been subjected to heating to elevated temperatures.

7. As a new article of manufacture, a rubber covered insulated wire comprising a wire having a coating of rubber insulating the same, and a textile covering member applied to and covering the rubber coating, said textile covering member being impregnated with a bituminous impregnant, and having a bituminous finishing coating applied over and covering the textile covering, 15 said bituminous finishing coating being characterized by the ability when exposed to direct flame of forming a carbonaceous ash film on the surface thereof in sufficient amount to form an effective air seal to thereby prevent rapid propagation of flame, said finishing coating comprising a bituminous material selected from the group consisting of those natural asphalts, gilsonite, steam reduced and air blown asphalts from petroleum residua, coal tar pitches, stearine pitches, and mixtures thereof which are characterized by their non-

greasy and non-oily appearance and feel, and having incorporated therein at least one metallic soap insoluble in water and comprising a soap selected from the soaps of the group of metals consisting of iron, zinc, aluminum, and barium, in an amount not exceeding fifteen per cent by weight of the bituminous composition, said flame retarding bituminous composition being further characterized by its ability to maintain substantially predetermined physical characteristics upon cooling after having been subjected to heating to elevated temperatures.

8. As a new article of manufacture, a rubber covered insulated wire comprising a wire having a coating of rubber insulating the same, and a textile covering member applied to and covering the rubber coating, said textile covering member being impregnated with a bituminous impregnant, and having a bituminous finishing coating applied over and covering the textile covering, said bituminous finishing coating being characterized by the ability when exposed to direct flame of forming a carbonaceous ash film on the surface thereof in sufficient amount to form an effective air seal to thereby prevent rapid propagation of flame, said impregnant and said finishing coating each comprising bituminous materials selected from the group consisting of those natural asphalts, gilsonite, steam reduced and air blown asphalts from petroleum residua, coal tar pitches, stearine pitches, and mixtures thereof which are characterized by their non-greasy and non-oily appearance and feel, and having incorporated therein at least one metallic soap insoluble in water and comprising a soap selected from the soaps of the group of metals consisting of manganese, iron, zinc, chromium, cobalt, magnesium, lead and barium, in an amount not exceeding fifteen per cent by weight of the bituminous composition, said flame retarding bituminous composition being further characterized by its ability to maintain substantially predetermined physical characteristics upon cooling after having been subjected to heating to elevated temperatures.

9. As a new article of manufacture, a rubber covered insulated wire comprising a wire having a coating of rubber insulating the same, and a textile covering member applied to and covering the rubber coating, said textile covering member being impregnated with a bituminous impregnant, and having a bituminous finishing coating applied over and covering the textile covering, said bituminous finishing coating being characterized by the ability when exposed to direct flame of forming a carbonaceous ash film on the surface thereof in sufficient amount to form an effective air seal to thereby prevent rapid propagation of flame, said finishing coating comprising a bituminous material having a melting point between 170° F. and 300° F. and a hardness between 3 and 18 both measured in the manner described and being selected from the group consisting of those natural asphalts, gilsonite, steam reduced and air blown asphalts from petroleum residua, coal tar pitches, stearine pitches, and mixtures thereof which are characterized by their non-greasy and non-oily appearance and feel, and having incorporated therein at least one metallic soap insoluble in water and comprising a soap selected from the soaps of the group of metals consisting of iron, zinc, aluminum, and barium, in an amount not exceeding fifteen per cent by weight of the bituminous composition, said flame retarding bituminous composition be-

ing further characterized by its ability to maintain substantially predetermined physical characteristics upon cooling after having been subjected to heating to elevated temperatures.

- 5 10. As a new article of manufacture, a rubber covered insulated wire comprising a wire having a coating of rubber insulating the same, and a textile covering member applied to and covering the rubber coating, said textile covering member being impregnated with a bituminous impregnant, and having a bituminous finishing coating applied over and covering the textile covering, said bituminous finishing coating being characterized by the ability when exposed to direct flame of forming a carbonaceous ash film on the surface thereof in sufficient amount to form an effective air seal to thereby prevent rapid propagation of flame, said finishing coating comprising a bituminous material having a melting point between 170° F. and 300° F. and a hardness between 3 and 18 and said impregnant comprising a bituminous material having a melting point of from 100 to 200° F. and a hardness between 15 and 30, both being measured according to the described methods, said bituminous impregnant and said finishing coating each comprising a bituminous material selected from the group consisting of those natural asphalts, gilsonite, steam reduced and air blown asphalts from petroleum residua, coal tar pitches, stearine pitches, and mixtures thereof which are characterized by their non-greasy and non-oily appearance and feel, and having incorporated therein at least one metallic soap insoluble in water and comprising a soap selected from the soaps of the group of metals consisting of iron, zinc, aluminum, and barium, in an amount not exceeding fifteen per cent by weight of the bituminous composition, said flame retarding bituminous composition being further characterized by its ability to maintain substantially predetermined physical characteristics upon cooling after having been subjected to heating to elevated temperatures.
- 15 20 25 30 35 40 45 50 55 60 65 70 75 11. As a new article of manufacture, a rubber covered insulated wire comprising a wire having a coating of rubber insulating the same, and a textile covering member applied to and covering the rubber coating, said textile covering member being impregnated with a bituminous impregnant, and having a bituminous finishing coating applied over and covering the textile covering, said bituminous finishing coating being characterized by the ability when exposed to direct flame of forming a carbonaceous ash film on the surface thereof in sufficient amount to form an effective air seal to thereby prevent rapid propagation of flame, said finishing coating comprising a bituminous material having a melting point between 170° F. and 300° F. and a hardness between 3 and 18 both measured in the manner described and being selected from the group consisting of those natural asphalts, gilsonite, steam reduced and air blown asphalts from petroleum residua, coal tar pitches, stearine pitches, and mixtures thereof which are characterized by their non-greasy and non-oily appearance and feel, and having incorporated therein at least one metallic soap insoluble in water and comprising a soap selected from the soaps of the group of metals consisting of manganese, iron, zinc, chromium, cobalt, aluminum, magnesium, lead and barium, in an amount not exceeding fifteen per cent by weight of the bituminous composition, said flame retarding bituminous compo-

sition being further characterized by its ability to maintain substantially predetermined physical characteristics upon cooling after having been subjected to heating to elevated temperatures.

12. As a new article of manufacture, a rubber covered insulated wire comprising a wire having a coating of rubber insulating the same, and a textile covering member applied to and covering the rubber coating, said textile covering member being impregnated with a bituminous impregnant, and having a flame retarding bituminous composition applied over and covering the textile covering, said composition possessing the property when exposed to direct flame of forming on the surface thereof a carbonaceous ash film of sufficient density and in sufficient amount to form an effective air seal covering the underlying bituminous material to thereby

prevent rapid propagation of flame, comprising a bituminous material selected from the group consisting of those natural asphalts, gilsonite, steam reduced and air blown asphalts from petroleum residua, coal tar pitches, stearine pitches, and mixtures thereof which are characterized by their non-greasy and non-oily appearance and feel, and having incorporated therein a mixture of zinc, barium, and aluminum soaps in an amount not exceeding fifteen per cent by weight of the bituminous composition, said flame retarding bituminous composition being further characterized by its ability to maintain substantially predetermined physical characteristics upon cooling after having been subjected to heating to elevated temperatures.

PURDUM M. SNYDER.